

July 1, 1947.

A. W. ANISH ET AL

2,423,217

PHOTOGRAPHIC EMULSIONS CONTAINING SENSITIZING DYES

Original Filed Aug. 16, 1944

3,3'-DIETHYL-5,6-5',6'-DICYCLOHEXYLIDENEDIOXY-BENZTHIOPHOCYANINE IODIDE

*Fig. 1.*



3,3'-DIETHYL-5,6-CYCLOHEXYLIDENEDIOXY-5',6'-METHYLEDIOXY-BENZTHIOPHOCYANINE IODIDE

*Fig. 2.*



3,3'-DIETHYL-5,6-CYCLOHEXYLIDENEDIOXY-5',6'-METHYLEDIOXY-BENZTHIOPHOCYANINE IODIDE

*Fig. 3.*



3,3'-DIETHYL-5,6-5',6'-DICYCLOPENTYLIDENEDIOXY-BENZTHIOPHOCYANINE IODIDE

*Fig. 4.*



3,3'-DIETHYL-5,6-CYCLOHEXYLIDENEDIOXY-5',6'-BENZOBENZTHIOPHOCYANINE IODIDE

*Fig. 5.*



3,3'-DIETHYL-5,6-CYCLOHEXYLIDENEDIOXY-5',6'-DIMETHOXYBENZTHIOPHOCYANINE IODIDE

*Fig. 6.*



*Inventors*  
Alfred W. Anish.  
Lee C. Hensley.

*By* *George W. Coughlin*  
*Attorneys.*

## UNITED STATES PATENT OFFICE

2,423,217

PHOTOGRAPHIC EMULSIONS CONTAINING  
SENSITIZING DYES

Alfred W. Anish, Johnson City, and Lee C. Hensley, Binghamton, N. Y., assignors to General Aniline & Film Corporation, New York, N. Y., a corporation of Delaware

Original application August 16, 1944, Serial No. 549,788. Divided and this application August 16, 1944, Serial No. 549,790

4 Claims. (Cl. 95—7)

1

The present invention relates to the sensitizing of photographic emulsions with new compounds of the thio and seleno-carbocyanine type.

In certain processes of subtractive multi-color photography a multi-layer photographic material is used in which the lowest light-sensitive layer is sensitive only for red above 6000 A. U. This red-sensitive layer must always be insensitive to blue-green light since the presence of blue-green sensitivity gives rise to falsification of color. In all color-photography processes in which the color of the component picture is produced by color development, there may be present in the photographic layer in addition to the sensitizer a color former which, when the exposed silver halide emulsion is developed, combines with the oxidation product of the developer to form a sparingly soluble dye distributed in the layer proportionately to the quantity of silver image. In this case, a sensitizer must be selected, the effect of which is not enfeebled by the presence of the dye component. Sensitizers are already known which have a high intensity in the red region of the spectrum but, these for the most part are enfeebled by the presence of a dye component.

It is known that many carbocyanines, of which the 5,6-position of the benzene nucleus is occupied, sensitize photographic silver halide emulsions to high red sensitivity. Most of these carbocyanines, however, are not suitable for sensitizing silver halide emulsions containing color coupling components. This is thought to be due to a physical displacement which the sensitizing dye undergoes when color coupling components are added. That is, the sensitizer is adsorbed to the surface of the silver halide grain, and then, with addition of color component, is displaced therefrom.

An object of the present invention is to provide a class of sensitizers which are free from the disadvantages noted above.

A further object is to provide a new class of thio and seleno-carbocyanines which are added to photographic emulsions, or coated thereon as an overcoating, whereby the sensitivity of the photographic emulsion is increased.

A still further object is to provide sensitizing dyes which are unaffected by the color forming development components.

Other objects and advantages of this invention will become apparent by reference to the following specification in which its preferred details and embodiments are described.

This invention is based on the discovery that thio and seleno-carbocyanines containing a cy-

2

clic hydrocarbon substituted dioxy ring structure as part of the cyanine dye molecule not only sensitize a photographic silver halide emulsion to high red sensitivity, but are also compatible with color coupling components for the cyan dye image. In the latter combination the sensitizing action of the dyes is not impaired or diminished. In addition to these desirable characteristics, it has been further found that when used in conjunction with color coupling components for the blue-green image, the spectral curves of these dyes show a desirable gap in the green region of the spectrum—that is, the dye sensitivity is more selective to the red spectral region. The sensitizing capacity of these dyes is not only maintained in the presence of color formers for the blue-green image, especially those color formers containing long chain hydroxyalkyl groups, but is increased, and in part rendered more selective. This entirely new property is most surprising and wholly unexpected. An additional advantage of these dyes is their ability to remain fixed in the one layer in which they are originally deposited.

The sensitizing dyes suitable for the purpose of the present invention have the general formula:



35 wherein R represents the methylene groups necessary to complete at least a 5-membered alicyclic system such as cyclopentylidene, cyclohexylidene, cycloheptylidene and the like, R<sub>1</sub> and R<sub>2</sub> are alkyl groups, e. g., methyl, ethyl, propyl, butyl, pentyl, etc., Y represents sulfur or selenium, X represents an acid radical, e. g., Cl, Br, I, SO<sub>4</sub>, ClO<sub>4</sub>, SO<sub>4</sub>CH<sub>3</sub>, SO<sub>4</sub>C<sub>2</sub>H<sub>5</sub>, SO<sub>3</sub>C<sub>6</sub>H<sub>4</sub>CH<sub>3</sub>, and the like, and Z represents a grouping of molecules necessary to complete a heterocyclic ring usual in the cyanine dye art, such as indolenine, thiazole, benzthiazole, benzelenazole and the like; these rings may be substituted by alkyl as above, aryl, e. g., phenyl, naphthyl or anthranyl, hydrogenated ring system of the same values as R, alkoxy, e. g., methoxy, ethoxy, propoxy, butoxy, etc., alkyldioxy or cycloalkyldioxy nuclei.

These sensitizing dyes are obtained by condensing quaternary ammonium salts of thiazoles and selenazoles containing an alicyclic dioxy ring such as cyclopentylidenedioxy, cyclohexyl-

idenedioxy, or cycloheptylidenedioxy ring as part of the nucleus with ethyl-orthoformate or with 2-( $\beta$ -acetanilido vinyl)-5,6-methylenedioxybenzthiazole ethiodide, 2-( $\beta$ -acetanilido vinyl)-5,6-cyclohexylenedioxybenzthiazole ethiodide, or the corresponding seleno derivatives thereof.

The alicyclicdioxobenzenes used in preparing the alicyclicdioxobenzthiazoles and alicyclicdioxobenzselenazoles which are condensed with any one of the above listed intermediates or coupling agents, are readily prepared by reacting catechol with a cyclic ketone as described in Recueil Travaux Chimiques des Pays Bas, vol. 54, p. 997 (1935).

The following examples describe in detail the methods for accomplishing the above objects, but it is to be understood that they are inserted merely for the purpose of illustration, and are not to be construed as limiting the scope of the invention.

*Example I*

3,3'-diethyl-5,6-5',6'-dicyclohexylenedioxybenzthiocarbocyanine iodide



Cyclohexylenedioxybenzene was prepared according to the above publication by dissolving 55 gms. of catechol in 100 gms. of hot anhydrous

Nine gms. of the disulfide were added to a mixture consisting of 28 cc. of acetic anhydride, 22 cc. of glacial acetic acid and 3 cc. of acetyl chloride, and heated on a steam bath. Eleven gms. of zinc dust were then added in small portions with stirring to the heated mixture. The free base was precipitated from the acid reaction mixture by pouring into 6 volumes of cold water. The 2-methyl-5,6-cyclohexylenedioxybenzthiazole was filtered, dried and had a melting point of 140-142° C. The ethyl-p-toluenesulfonate salt was made in the usual manner and had a melting point of 169° C.

0.69 gm. of the quaternary salt thus prepared was treated with 0.5 cc. of ethyl-orthoformate in 5 gms. of pyridine in the presence of a trace of triethylamine at 130-140° C. for 3 hours. Upon cooling, 20 cc. of water was added. After standing overnight, the solid that separated was dissolved in 15 cc. of hot n-propyl alcohol and the solution treated with 3 cc. of 20% potassium iodide solution, filtered and allowed to cool. The dye precipitated on standing. It was filtered off, and after washing with water, the dye was recrystallized from ethyl alcohol as the iodide. The crystals melted above 250° C.

Incorporated in a gelatino silver halide emulsion containing about 4-5% of silver halide, the dye sensitized to about 6800 Å., with a maximum sensitivity of 6400 Å.

Twenty milligrams of the sensitizing dye prepared as above were dissolved in 50 cc. of methyl alcohol, and added to a kilo of silver halide gelatin emulsion containing about 10% gelatin, 4-5% of silver halide and 12.0 gms. of N-octadecyl-1-hydroxy-2-naphthoylamine. The coated emulsion had a maximum red sensitivity at about 6650 Å., and developed to a blue-green image with p-phenylenediamine developer. The sensitizing dye did not diffuse in multi-layer coatings.

*Example II*

3,3'-diethyl-5,6-cyclohexylenedioxy-5',6'-methylenedioxybenzthiocarbocyanine iodide



cyclohexanone and treated with an excess of phosphoric anhydride (125 gms.). After the addition was completed, the stirring was continued for a short time, and the upper layer decanted. The decanted material was mixed with 150 cc. of a dilute solution of sodium carbonate and steam-distilled. The distillate was extracted with ether and the dried solvent evaporated. The residue of the cyclohexylenedioxybenzene was distilled at reduced pressure and the resulting distillate had a boiling point of 125° C. at 12 mm. M. P. 44° C.

The cyclohexylenedioxybenzene was converted to 1,2-dinitro-4,5-cyclohexylenedioxybenzene by treating the former with a mixture of glacial acetic and fuming nitric acids. The resulting product was then converted to the disulfide by treating it in 200 cc. of boiling ethyl alcohol with a fused mixture of equivalent quantities of sodium sulfide nonahydrate and sulfur in small portions until a violet color persisted for a few minutes. The solid was filtered from the cool mixture, washed alternately with water and alcohol, and dried.

250 milligrams of 2-( $\beta$ -acetanilido vinyl)-5,6-methylenedioxybenzthiazole ethiodide prepared by heating at 135° C. a mixture of equal weight portions of 2-methyl-5,6-methylenedioxybenzthiazole ethiodide and diphenyl formamidine in acetic anhydride for 40 minutes, were mixed with an equal amount of 2-methyl-5,6-cyclohexylenedioxybenzthiazole ethyl-p-toluenesulfonate prepared according to Example I, in 5 cc. of pyridine and 3 drops of triethylamine. The mixture was heated to reflux for 1 hour, cooled, and an equal volume of water added. The dye crystals which separated out on standing were filtered off and recrystallized from ethyl alcohol.

Incorporated in a gelatino silver halide emulsion containing about 4-5% of silver halide, the dye sensitized to about 6850 Å., with a maximum sensitivity at 6420 Å.

Twenty-five milligrams of the sensitizing dye above prepared were dissolved in 50 cc. of methyl alcohol, and added to a kilo of silver halide gelatin emulsion containing about 10% gelatin, 4-5% of silver halide, and 12 gms. of 3,5-di(phenylamino)phenol. The coated emulsion showed a

high red sensitivity, and developed to a blue-green image with a p-phenylenediamine developer.

*Example III*

3,3'-diethyl-5,6-cyclohexylidenedioxy-5',6'-methylenedioxy-benzthiobenzselenocarbocyanine iodide



0.8 gm. of 2-( $\beta$ -acetanilido vinyl)-5,6-cyclohexylidenedioxybenzthiazole ethiodide and 0.6 gm. of 2-methyl-5,6-methylenedioxybenzselena-azole ethyl-p-toluenesulphonate were mixed with 25 cc. of pyridine and 0.5 cc. of triethylamine added. The mixture was refluxed for 1 $\frac{1}{2}$  hours. The dye solution was diluted with water and allowed to stand overnight. The dye crystals which separated were filtered off and washed with water, and recrystallized from ethyl alcohol.

Incorporated in a gelatino silver halide emulsion containing about 4-5% of silver halide, the dye sensitized to about 6850 A., with a maximum sensitivity at 6450 A.

Twenty-five milligrams of the sensitizing dye prepared as above were added to a kilo of silver halide gelatin emulsion containing about 10% gelatin, 4-5% of silver halide and 12.0 gms. of N-octadecyl-1-hydroxy-2-naphthoylamine. The coated emulsion showed a high red sensitivity, and developed to a blue-green image with a p-phenylenediamine developer. The dye did not diffuse in multi-layer coatings.

When 8.0 gms. of 1-hydroxy-2,4-dichloronaphthalene were substituted for 12.0 gms of N-octadecyl-1-hydroxy-2-naphthoylamine, the coated emulsion showed a high red sensitivity, and developed to a blue-green image with a p-phenylenediamine developer.

*Example IV*

3,3'-diethyl-5,6-5',6'-dicyclopentylidenedioxy-benzthiocarbocyanine iodide



5.3 gms. of 2-methyl-5,6-cyclopentylidenedioxybenzthiazole ethyl-p-toluenesulfonate, prepared in a manner similar to the corresponding 2-methyl-5,6-cyclohexylidenedioxybenzthiazole in Example I, and five gms. of ethyl-orthoformate were refluxed in 20.0 cc. of pyridine for 2 $\frac{1}{2}$  hours. An equal volume of water was added and the dye which separated was filtered off, washed with water, and crystallized from methyl alcohol.

Incorporated in a gelatino silver halide emulsion containing 4-5% of silver halide, the dye sensitized to about 6800 A., with a maximum sensitivity at 6400 A.

Twenty-five milligrams of the sensitizing dye prepared as above were added to a kilo of silver halide gelatin emulsion containing about 10% gelatin, 4-5% of silver halide, and 10 gms. of 8-hydroxyquinoline as the color former. The coated emulsion showed a high red sensitivity, and de-

veloped to a blue-green image with a p-phenylenediamine developer.

*Example V*

3,3'-diethyl-5,6-cyclohexylidenedioxy-5',6'-benzobenzthiocarbocyanine iodide



- 15 0.8 gm. of 2-( $\beta$ -acetanilido vinyl)-5,6-cyclohexylidenedioxybenzthiazole ethiodide were mixed with 4.0 gms. of 2-methyl-6,7-benzobenzothiazole ethyl-p-toluenesulfonate, 20.0 cc. pyridine and 4.0 cc. triethylamine. The mixture was heated to reflux for one hour, cooled, and an equal volume of water added. The dye crystals which separated out on standing were filtered off and recrystallized from methyl alcohol.
- 20 5.4 gms. of 2-( $\beta$ -acetanilido vinyl)-5,6-cyclohexylidenedioxybenzthiazole ethiodide were mixed with 4.0 gms. of 2-methyl-6,7-benzobenzothiazole ethyl-p-toluenesulfonate, 20.0 cc. pyridine and 4.0 cc. triethylamine. The mixture was heated to reflux for one hour, cooled, and an equal volume of water added. The dye crystals which separated out on standing were filtered off and recrystallized from methyl alcohol.
- 25 Incorporated in a gelatino silver halide emulsion containing 4-5% of silver halide, the dye sensitized to about 6800 A., with a maximum sensitivity at 6400 A.

- 30 35 Twenty-five milligrams of the sensitizing dye prepared as above were added to a kilo of silver halide gelatin emulsion, containing about 10% gelatin, 4-5% of silver halide, and 10 gms. of o-hydroxydiphenyl as the color former. The coated emulsion showed a high red sensitivity.
- 40 Twenty-five milligrams of the sensitizing dye prepared as above were added to a kilo of silver halide gelatin emulsion, containing about 10% gelatin, 4-5% of silver halide, and 10 gms. of o-hydroxydiphenyl as the color former. The coated emulsion showed a high red sensitivity.

*Example IV*

3,3'-diethyl-5,6-5',6'-dicyclopentylidenedioxy-benzthiocarbocyanine iodide



and developed to a blue-green image with a p-phenylenediamine developer.

*Example VI*

3,3'-diethyl-5,6-cyclohexylidenedioxy-5',6'-dimethoxybenzothiocarbocyanine iodide



- 60 75 5.4 gms. of 2-( $\beta$ -acetanilido vinyl)-5,6-cyclohexylidenedioxybenzthiazole ethiodide was mixed with 4.2 gms. of 2-methyl-5,6-dimethoxybenzothiazole ethyl-p-toluenesulfonate, 20 cc. of pyridine and 4 cc. of triethylamine. The mixture was heated to reflux for one hour, cooled, and an equal amount of water added. The dye crystals which

separated out on standing were filtered off and recrystallized from methyl alcohol.

Incorporated in a gelatino silver halide emulsion containing about 4-5% of silver halide, the dye sensitized to about 6800 Å, with a maximum sensitivity at 6400 Å.

Twenty-five milligrams of the sensitizing dye prepared as above were added to a kilo of silver halide gelatin emulsion containing about 10% gelatin, 4-5% of silver halide, and 12 gms. of 10 α-hydroxy naphthoic acid as the color former. The coated emulsion showed a high red sensitivity, and developed to a blue-green image with a p-phenylenediamine developer.

The diagrammatic spectrograms constituting the accompanying drawing illustrate the regions of the spectrum to which the various types of thio- and seleno-carbocyanines containing a cyclic hydrocarbon substituted dioxy ring structure as part of the cyanine dye molecule disposed herein will sensitize a gelatino silver-halide emulsion containing about 4-5% of silver halide and the extent of the sensitization at various wave lengths. The six figures of this drawing illustrate the sensitizing properties of the dyes prepared in accordance with the preceding examples.

In the preparation of silver halide emulsions containing the sensitizing dyes of the present invention, the dyes may be dissolved in methyl or ethyl alcohol and a volume solution containing from 5 to 50 milligrams of the dye added to a liter of emulsion. While in general practice it may not be necessary to add the dye in larger amounts, generally, for satisfactory results, amounts usually ranging from 5 to 25 milligrams are sufficient to obtain the maximum sensitizing effect. However, we do not wish to limit our invention to the quantities just indicated; the most suitable amount will in each case be found by a few comparative experiments. The dyes may be added to the emulsion in form of solutions. In actual practice, the dyes are applied to the emulsion during any stage of its production; however, they are preferably added to the finished emulsion before being cast.

This application is a division of our co-pending application Serial No. 549,788 filed on even date.

The above examples are illustrative only, and should not be construed as limiting the invention, since it will be apparent to those skilled in the art, that the sensitizers may be incorporated into photographic emulsions by methods other than those described herein.

While there have been pointed out above certain preferred embodiments of the invention, the same is not limited to the foregoing examples, illustrations, or to the specific details given therein, but is capable of variations and modifications as to the reactants, proportions and conditions employed. Accordingly, it is intended that the invention be defined only by the accompanying claims.

We claim:

1. A photographic gelatino-silver-halide emulsion which contains 3,3'-diethyl-5,6,5',6'-dicyclohexylienedioxybenzthiocarbocyanine iodide.

2. A photographic gelatino-silver-halide emulsion which contains 3,3'-diethyl-5,6-5',6'-dicyclopentylienedioxybenzthiocarbocyanine iodide.

3. A photographic gelatino-silver-halide emulsion which contains 3,3'-diethyl-5,6-cyclohexylienedioxy-4',5'-methylenebenzselenothiazolocarbocyanine iodide.

4. A photographic gelatino-silver-halide emulsion which contains a sensitizing dye of the general formula:



wherein R represents the methylene groups necessary to complete at least a 5-membered alicyclic system, R<sub>1</sub> and R<sub>2</sub> represent an alkyl group, X represents an acid radical, Y represents a member taken from the class consisting of sulfur and selenium, and Z represents the atoms necessary to complete a nitrogenous heterocyclic ring system.

ALFRED W. ANISH,  
LEE C. HENSLEY.

#### REFERENCES CITED

The following references are of record in the file of this patent:

#### UNITED STATES PATENTS

| Number    | Name            | Date          |
|-----------|-----------------|---------------|
| 2,126,078 | Zeh et al.      | Aug. 9, 1938  |
| 2,104,855 | Dieterle et al. | Jan. 11, 1938 |

#### FOREIGN PATENTS

| Number  | Country       | Date          |
|---------|---------------|---------------|
| 425,417 | Great Britain | Mar. 14, 1935 |

**Certificate of Correction**

Patent No. 2,423,217.

July 1, 1947.

**ALFRED W. ANISH ET AL.**

It is hereby certified that errors appear in the printed specification of the above numbered patent requiring correction as follows: Column 5, Example III, in the formula, extreme right hand portion thereof, for "S" read *Se*; line 32, for "4-5" read 4-5%; column 7, line 7, for "miliigrams" read *milligrams*; and that the said Letters Patent should be read with these corrections therein that the same may conform to the record of the case in the Patent Office.

Signed and sealed this 21st day of October, A. D. 1947.

[~~SEAL~~]

**THOMAS F. MURPHY,**  
*Assistant Commissioner of Patents.*